

[54] **METHOD OF FORGING SINTERED ARTICLES OF HIGH DENSITY**

[76] Inventor: **Saburo Goto, 49-Banchi, Shichiku Kamiumenoki-cho, Kita-ku, Kyoto, Japan**

[22] Filed: **Jan. 21, 1972**

[21] Appl. No.: **219,652**

[30] **Foreign Application Priority Data**

Oct. 7, 1971 Japan..... 46-78909

[52] **U.S. Cl.** ..... 72/342, 29/420.5

[51] **Int. Cl.** ..... B21j 1/06

[58] **Field of Search** ..... 29/420.5, DIG. 31; 72/342

[56] **References Cited**

UNITED STATES PATENTS

2,757,446 8/1956 Boegehold et al. .... 29/420.5

|           |        |                     |          |
|-----------|--------|---------------------|----------|
| 2,821,016 | 1/1958 | Dickson .....       | 72/342   |
| 3,645,728 | 2/1972 | Hrinevich, Jr. .... | 29/420.5 |
| 3,605,245 | 9/1971 | Zapf.....           | 29/420.5 |

*Primary Examiner*—Lowell A. Larson  
*Attorney, Agent, or Firm*—Wenderoth, Lind & Ponack

[57] **ABSTRACT**

A method of forging sintered articles of high density characterized in that pre-shaped powdery articles are heated to a temperature of 1120°-1200°C and then are forged by a tool, which is pre-warmed to 80°-120°C and maintained at such pre-warming temperature, at a tool speed of 7-10m/second. The articles thus forged are rapidly separated from the tool through the medium of an ejector provided on the forging machine.

**3 Claims, 1 Drawing Figure**

PATENTED MAR 5 1974

3,795,129



# METHOD OF FORGING SINTERED ARTICLES OF HIGH DENSITY

## BACKGROUND OF THE INVENTION

This invention relates to a method of forging whereby the necessity of the precise forged articles of high density can be produced without re-sintering process of moulding.

This invention is characterized in that powdery articles, pre-shaped by a conventional method or by a specific method, are heated to a temperature of 1120° – 1200°C, while a tool is pre-warmed to a temperature of from 80° to 120°C and is maintained at this pre-warming temperature. The heated articles then are forged in the tool at a speed of 7 – 10m/second. forging, the finished forged article and the tool are separated rapidly by a separating apparatus provided on the forging machine.

High density is essential for sintered articles such as forged machine parts. In this respect, U.S. Pat. No. 3,410,683 discloses the method whereby a molded article is heated to a temperature of about 750°C – 1100°C before it is re-pressed, and the press tool is pre-warmed to a temperature of 150°C – 350°C and is maintained at this pre-warming temperature throughout the re-pressing operation, in order to keep the recrystallisation conditions of the article during re-processing constant. It appears that the purpose of this method is to obtain precise finished articles by maintaining the temperature of the press tool high and by maintaining the temperature of article low or from 750°C to 1100°C so as to reduce the temperature difference between the tool and the material, thereby avoiding temperature drop of the article as far as possible and thus increasing the fluidity of the material. However, the lower temperature of the actually material results in lowering the fluidity and consequently lowering the degree of precision of the finished article. Moreover, since the press tool is bulky, it is extremely difficult to maintain its temperature high.

The most important problem raised in hot forging is that during the processing of a highly heated article on the press tool, the surface temperature of the tool rises and the surface of tool is transformed due to thermal fatigue and wear. A finished article, after separation from the tool, is cooled by compulsory cooling but it is difficult to prevent the rising of its temperature due to conduction of heat at the contact surface with the tool during processing. Thus, the best way for forging a powdery substance is to process the heated substance as quickly as possible. Furthermore, a faster tool speed and a shorter processing time improve the flow of the material of a preshaped sintered article, decrease the coefficient of kinetic friction and effect the uniform distribution of pressing force into every part of the finished article, with the result of uniform density. The forging machine primarily used is an oil-pressure forging press of low processing speed (0.6m/second or lower). Presses such as the drop hammer, friction press, etc., work at the medium speed or 2 – 4m/second, and a forging machine of the upward pressurizing type works at the high speed of 7 – 10m/second.

As is obvious from the foregoing, the time during which the tool makes contact with a heated article decreases in inverse proportion to the tool speed. Therefore, when using a forging machine of low speed, the

temperature of the tool must be kept at least as high as 150 – 350°C, or otherwise the article undergoes a large temperature drop at the area in contact with the tool, with the result of uneven density due to the partial difference in cooling speed. On the other hand, when a forging machine with a high processing speed, such as DYNAPACK, is used, the wear of the tool is large due to the longer time required for separation, even though the operating speed is high (12 – 19m/second).

## SUMMARY OF THE INVENTION

In the present invention, a forging machine having a high processing speed and a shorter tool separation time is used, for example, a forging machine of the KJH series. This type of forging machine belongs to the group of hammering machines of the upward pressurizing type. It works at a speed of 7 – 10m/second and is equipped with a tool separating apparatus such as an ejector. It provides optimum conditions for obtaining the uniformly high density of the powdery article during forging because of the synchronization of the dropping of an upper tool and the rising of a lower tool. In the present invention, a lubricant may be applied to the tool, instead of adding a lubricant to the powdery substance.

## BRIEF DESCRIPTION OF THE DRAWINGS

The single FIGURE is a microscopic photograph of a finished article forged in accordance with the present invention.

## EXAMPLE OF INVENTION

The result of test forging carried out by using the above discussed forging machine in accordance with the temperature and other limitations of the process of this invention was as follows:

|                      |                                             |
|----------------------|---------------------------------------------|
| Forging conditions:  |                                             |
| Pre-shaped powder:   | Electrolytic iron powder                    |
| Forging temperature: | Pressed powder density: 6.8/cm <sup>3</sup> |
| Heating duration:    | 1180°C                                      |
| Processing energy:   | 30 minutes (hydrogen atmosphere)            |
|                      | 0.7 ton – m                                 |

Finished articles forged under the above conditions were examined for physical properties with a microscopic photograph (200 magnifications), per the attached drawing, with the following results.

|    | Density<br>g/cc | Tensile<br>strength<br>kg/mm <sup>2</sup> | Elongation<br>% | Charpy<br>impact value<br>Kgm/cm <sup>2</sup> |
|----|-----------------|-------------------------------------------|-----------------|-----------------------------------------------|
| 50 | 7.85            | 26.24                                     | 55.7            | 30 or more                                    |

As is obvious from the above test results, forged articles produced according to the present invention exhibit superior physical properties to conventionally forged articles.

What is claimed is:

1. A method for forging a sintered article having a high density, said method comprising:  
pre-heating to a temperature of 80°–120°C the forging tool of a forging machine of the type having an upper element and a lower element movable together in synchronization;  
heating a pre-shaped powdery article to a temperature of 1120°–1200°C;  
forging said heated pre-shaped powdery article by said pre-heated tool at a forging operating speed of

7-10 m/second, while maintaining said tool at the preheating temperature; and separating the thus forged article from said tool by operating an ejector device positioned on said forging machine.

2. A method as claimed in claim 1, wherein said for-

ing is accomplished by a synchronized lowering of said upper element and raising of said lower element.

3. A method as claimed in claim 1, wherein said pre-shaped powdery article is heated to a temperature of 5 1180°-1200°C.

\* \* \* \* \*

10

15

20

25

30

35

40

45

50

55

60

65